

## UNITED STATES PATENT OFFICE

2,237,485

PROCESS FOR THE DEOXIDATION AND  
DEGASIFICATION OF STEEL

Paul Hardt, Volklingen-Saar, Germany, assignor  
to Röchling'sche Eisen- und Stahlwerke Gesell-  
schaft mit beschränkter Haftung, Volklingen-  
Saar, Germany, a limited-liability company

No Drawing. Application May 2, 1939, Serial No.  
271,342. In Germany May 7, 1938

## 2 Claims. (CL 75—57)

It is a known fact, that carbon is unsuitable for the deoxidation of soft steel, because small quantities of carbon remain ineffective, whereas large quantities increase the carbon content of the steel. The use of a carbonizing liquid consisting of tar, oil, wax, paraffin or pitch for increasing the carbon content of ingot iron or steel is also known.

It has been recognized according to the invention that, contrary to the statements in older patent literature, hydrocarbon of high molecular weight, especially pit coal pitch, has no or only very little carbonizing effect but a strong deoxidizing and degasification action when added to steel baths. Pit coal pitch has been found to be particularly effective when it is stiffened by an addition of pulverized burnt lime dust, silicates and fluxes. It is preferably used in the form of pressed or cast bricks.

The cause for the deoxidizing and degasification effects of pit coal pitch is partly due to the evaporating pitch forming over the steel bath heavy vapors which protect the bath against contact with the air. For example

|                                           | Kilograms |
|-------------------------------------------|-----------|
| 1 Nm <sup>3</sup> of air weighs           | 1.3       |
| 1 Nm <sup>3</sup> coke gas weighs         | 0.6       |
| 1 Nm <sup>3</sup> anthracene vapor weighs | 8.0       |

Nm<sup>3</sup> means cubic meter at normal conditions of temperature and pressure (0° C. and 760 m./m.Hg (mercury). Therefore, at a temperature of 1700° C. anthracene vapor still has the same specific gravity as air at 50° C., that is the temperature of the surroundings prevailing during

the casting. The steel is therefore always covered by a layer of pitch vapors.

Mixtures of pitch with pulverized burnt lime in a proportion of 1:3 have shown a strong deoxidizing effect. The lime addition may, however, be varied. For lowering the sintering temperature of the lime, silicates, fluor spar, soda and the like may be added. Preferably additions are used which themselves have a purifying effect on the steel. On the other hand substances such as finely pulverized ferro manganese, calcium carbide and the like may be added which have a reducing or deoxidizing effect. A particularly good effect is obtained, when the pitch or the mixture of pitch and lime is previously worked into lumps, shaped body or pressings. The pieces are thrown into the liquid steel when filling the ladle or can be added in the mold during the casting.

## I claim:

1. A process for the deoxidation and degasification of steel, consisting of treating the liquid steel with a mixture of pitch and dust of lime with the proportion of lime greater than the pitch, and silicates and other fluxes in an amount sufficient to lower the sintering temperature of the lime.
2. A process for the deoxidation and degasification of steel, consisting of introducing a mixture in the steel bath in cold form in which the mixture comprises pitch with dust of lime with the proportion of lime greater than the pitch and silicates and other fluxes in an amount sufficient to lower the sintering temperature of the lime.

PAUL HARDT.